

# UNITED STATES PATENT OFFICE.

HERMANN A. SEEGALL, OF BERLIN, GERMANY.

## PROCESS OF MAKING CHROMIUM SULPHATES.

SPECIFICATION forming part of Letters Patent No. 415,739, dated November 26, 1889.

Application filed March 25, 1889. Serial No. 304,682. (No specimens.)

*To all whom it may concern:*

Be it known that I, HERMANN ALBERT SEE-GALL, a subject of the King of Prussia, German Emperor, and a resident of 129 Invaliden 5 Strasse, Berlin, Germany, have invented certain new and useful Improvements in the Production of Chromium Sulphate, of which the following is a full and clear specification.

Up to the present the process of working 10 substances containing chromium in order to obtain a soluble preparation of that element consisted in oxidizing the material in question in order to obtain an alkali chromate or bichromate, which formed the groundwork of 15 all other chrome preparations. The disintegration of chrome ores for the purpose of analyzing the same has been effected in the laboratory by means of melting them together with alkali bisulphate. This method 20 is not, however, suitable for trade purposes, since in order to secure a complete disintegration of the ores a large excess of bisulphate is necessary, whereby through the development of sulphuric-acid vapors the lungs 25 of the workmen are injuriously affected and only an imperfect utilization of the bisulphate is attained.

I have discovered that two important 30 points in the process must be taken into account and carried out before the same can be employed with advantage for trade purposes. The first of these two points consists in holding the chrome materials in suspension in melted alkali during the heating 35 of the same, in order to impart to it a large surface of contact for the escaping sulphuric acid. The second of these important points is the regaining of the sulphuric-acid vapors (having escaped without having taken part 40 in the reaction) through condensation. These two points in the disintegration of the raw materials containing chrome combine to make my process capable of being used with advantage for industrial purposes.

45 By my method, hereinafter described, I am enabled to obtain a chromic sulphate in the form of a soluble chrome preparation direct from the raw materials, suitable for industrial purposes, which can then be worked on 50 the other chrome preparations.

I pulverize the substance containing the chromium and heat it in receptacles pro-

vided with mechanical stirring apparatus, together with an acid sulphate of a fixed alkali. During the ensuing disintegration 55 or decomposition of the raw materials, which is very complete in consequence of the thorough mixing of the ore with the sulphuric acid produced, a rather large quantity of vapors containing  $SO_3$  (and  $SO_2$ ) escapes. I 60 conduct these vapors by means of pipes into cooled condensers, where I obtain the sulphuric acid, while I take the remaining sulphurous acid into a receiver containing lime-milk and obtain there calcium hyposulphite. 65 The holding of the raw material in suspension during the heating, which is throughout necessary for the process, may not only be attained by means of stirring apparatus, but also by a shaking apparatus or revolving 70 furnace.

In the process just described the only disadvantages are the necessity of carrying on the heating in covered receptacles, of condensing the escaping gases, and of having to work 75 with a mechanical stirring arrangement of some sort.

I have further found that the quantity of the vapors produced during the heating or melting may be reduced to a minimum or entirely prevented if some quantity of a substance be introduced into the melted mass. The said substance must not melt or decompose at a temperature of  $600^{\circ}$  centigrade, but only serve to make the melted mass more 85 pulpy. The explanation of this result is the following:

Since the bisulphates of fixed alkalies melt to a pretty thin liquid at  $197^{\circ}$  centigrade, the powdered ore sinks to the bottom in the 90 liquid alkali bisulphate during the process on account of its heavier specific weight. In consequence the surface of contact of the two masses forms the only point where the bisulphate can exercise its influence on the ore. 95 At about  $340^{\circ}$  centigrade the bisulphate is converted into pyrosulphate and water,



and at  $600^{\circ}$  centigrade this salt decomposes into neutral sulphate and sulphuric-acid anhydride,



The sulphuric acid which becomes free can of course only work upon the ore on coming

into contact with the same. It cannot, however, come into contact with the ore if the same is lying on the bottom of the melting-pot and the sulphuric acid steaming away from the upper surface of the contents of the pot. It is here that the advantage becomes apparent of intermixing a substance which neither melts nor decomposes nor precipitates at a temperature of  $600^{\circ}$  centigrade.

10 The melted mass is no longer so thin and the powdered ore is no longer able to sink to the bottom, but is held in close contact with the melted bisulphate, and is in consequence subjected to the influence of the sulphuric acid released from the same. When the sulphuric acid has once combined, it will no longer escape at the temperature mentioned, and only those parts of the bisulphate which are lying right on the surface will give off their  $SO_3$ .

15 It is for this reason advisable to add a certain amount of the refractory substance to the melting mass. The gases can then with difficulty make their way through the pulpy mass in order to escape.

20 There are certainly some materials containing chromium (chrome slags) which when melted with bisulphate immediately cause the mass to assume a thick pulpy nature; but they do not remain suspended in the same, and in consequence require the aid of a mechanical stirring apparatus. If I take  $s$ , specific gravity of the substance added,  $P$  absolute weight of the substance added,  $s^2$  specific gravity of the mixture set,  $G$  weight of the mixture set or melted, and  $x$  equal the quotient of the volume of the mixture set by the volume of the melted mixture, then

25 
$$P = \frac{Gs'}{s^2}$$
 and  $x = \frac{s^3}{s^2}$ . If  $x$  equal one, no addition is necessary.

30 All substances which do not melt or decompose at the temperature necessary for the process—viz.,  $600^{\circ}$  centigrade—may be used for adding to the mixture, particularly the oxides, hydrated oxides, non-volatile salts of the metals of the alkaline earths, and of the earthy metals and silicic acid. In case it is not required to gain sulphuric acid as a by-product, as in the process at first described,

35 the condensers and stirring apparatus may be dispensed with. When mixing any of the substances just mentioned to the melting mass, the decomposition of the materials containing chromium will be attained in the lastly-described manner.

40 I perform the process at first described in the following manner: One hundred parts of chrome ore and four hundred parts of sodium bisulphate are ground up very fine and thoroughly mixed. The mixture is then heated in covered receptacles provided with a stirring apparatus to  $600^{\circ}$  centigrade for the space of about two to two and one-half hours, by which means the chrome ore, since it is held in suspension, will be almost entirely decomposed, and the amount of sulphuric acid corresponding to two hundred parts of bisul-

phate will be received in the condensers. The gases ( $SO_2$ ) not condensed in the condensing apparatus will be arrested by the lime-milk. <sup>70</sup> The melted mass is then cooled up and lixiviated with water.

I perform the second method by finely powdering and mixing one hundred parts of chrome ore with two hundred parts of sodium bisulphate and fifty parts of barium sulphate and then heating the mixture to a temperature of  $600^{\circ}$  centigrade for about two to two and one-half hours. The quantity of vapors produced by this method is so insignificant <sup>75</sup> that they may be allowed to escape. After the melting has taken place the mass will be removed from the melting-pot and lixiviated with water. If barium sulphate be not used, as an addition, the minimum amount of the <sup>80</sup> mass to be added may be obtained from the equation for  $P$ . In any case a material must be chosen which at  $600^{\circ}$  centigrade does not combine with the sulphuric acid set free. Should a material be employed for this purpose which does combine with the sulphuric acid which is released, it is then always necessary to add bisulphate enough to satiate the requirements of the material added and then be sufficient to decompose the materials <sup>85</sup> containing the chrome. Accordingly  $s$  will in this case represent the specific gravity of the combination of the material added with sulphuric acid.

From the chrome sulphate which is contained in combination with other sulphates in the watery solution resulting from both methods it is now easily possible to obtain the hydrated oxide of chromium through precipitation by means of the well-known reagents, (such as caustic alkalies, alkaline carbonates, magnesia, &c.,) when the hydrated oxide of chromium forms a porous easily-<sup>100</sup> oxidizable mass. This hydrated oxide of chromium is certainly in the most cases impurified by the presence of hydrated oxide of aluminium and hydrated oxide of iron, from which it can, however, easily be separated, (for instance, by washing.) This hydrated oxide of chromium forms a much better <sup>105</sup> essential element for producing the other chrome preparations than the alkali bichromate used up to the present in the industry for the same purpose. For forming chrome salts from this hydrated oxide of chromium <sup>110</sup> it is not necessary to make any reduction, as the hydrated oxide of chromium combines directly with acids to form salts of chromium. The oxidation for the formation of chromates can also be conveniently carried out, <sup>115</sup> since the hydrated oxide of chromium combines directly with bases forming the corresponding chromates. In the latter case the oxygen in co-operation with the impurifying hydrated oxides produces an advantageous <sup>120</sup> effect, while in the methods of carrying out the oxidation up to the present in use impurities had a reducing effect on the melting mass.

In working the oxidation according to my method not only a saving of time is effected, but also less firing material is required. It may be carried out much more easily and 5 with far simpler and less expensive apparatus. Lastly, a much more complete using up of the materials employed is attained than in those processes in use up to the present.

In the following claims I mean by the term 10 "acid sulphates of any fixed alkali" not only the combination  $RHSO_4$ , but all sulphates of fixed alkalies which with regard to the combination  $R_2SO_4$  contain an excess of sulphuric acid.

15 Having thus fully declared the nature of my said invention, what I claim, and desire to secure by Letters Patent of the United States, is—

1. The process of manufacturing chromic 20 or chromous sulphates from materials containing chrome by heating the said substances in covered receptacles with the acid sulphates of any fixed alkali, and holding the materials containing chrome continually in suspension in the melting mass by mechanical agitation, for the purpose and in the manner 25 substantially as described.

2. The process of manufacturing chromic or chromous sulphates from materials containing chrome by heating the said substances in covered receptacles with the acid sulphates of any fixed alkali, and holding the materials containing chrome continually in suspension in the melting mass by mechanical agitation, and then condensing the escaping 30 vapors and regaining the sulphuric acid which has not entered into the reaction, substantially as herein described.

3. The process of manufacturing chromic or chromous sulphates from materials containing chrome by heating the substances with the acid sulphates of any fixed alkali and with a refractory mass which does not decompose or melt under  $600^{\circ}$  in such a manner that sulphuric oxide ( $SO_3$ ) is liberated 40 and decomposes the materials containing chrome, substantially as described.

In witness whereof I have hereunto set my hand in presence of two witnesses.

HERMANN A. SEEGALL.

Witnesses:

B. ROI,  
THEODOR HEESE.